

1

3,222,119

## PROCESS FOR TREATING CELLULOSIC TEXTILE MATERIALS WITH BIS(BETA-METHOXYETHYL) SULFONE

Irving Tashlick, Springfield, and Scott H. Foster, Longmeadow, Mass., assignors to Monsanto Company, a corporation of Delaware  
 No Drawing. Filed Mar. 10, 1959, Ser. No. 798,339  
 1 Claim. (Cl. 8—116)

This invention relates to modified cellulosic textile materials. More particularly, the invention relates to a method of treating cellulosic textile materials to improve their properties of dimensional stability, "wash-and-wear," and wrinkle recovery without imparting a tendency toward chlorine retention after bleaching.

Various treating agents have been found useful for improving the dimensional stability and wrinkle recovery of cellulosic textile materials. However, the treating agents which are known to be effective in this application usually have one or more of the following undesirable features: toxicity, expense, or relative inefficiency of the treating agent, instability to hydrolysis and heat, tendency toward chlorine retention when the treated material is bleached, development of objectionable odors in the treated material, yellowing with aging, yellowing on exposure to heat of an iron, or yellowing on treatment with hypochlorite bleach.

One object of this invention is to provide means for improving the dimensional stability and wrinkle recovery of cellulosic textile materials.

Another object is to provide such means by the use of treating agents which lack the aforementioned undesirable features of the treating agents previously known to be effective in improving the dimensional stability and wrinkle recovery of cellulosic textile materials.

These and other objects are attained by treating a cellulosic textile material with a water-soluble bis(beta-hydroxyalkyl)sulfone or bis(beta-alkoxyalkyl)sulfone in the presence of an alkaline catalyst.

The following examples are given to illustrate the invention.

### Example I

An aqueous solution of 10% by weight of bis(beta-hydroxyethyl)sulfone and 3% by weight of sodium carbonate (both percentages based on the total weight of the solution) is padded on a cotton print cloth having a count of 80 x 80 to deposit in the cloth 10% by weight of the sulfone, based on the weight of the untreated cloth. The cloth is then dried at 220° F. for 3 minutes and cured at 310° F. for 4 minutes.

The treated cloth has a wrinkle recovery of 259° (warp plus filling), as determined by ASTM test method D1295-53T, compared to a wrinkle recovery of 100° (warp plus filling) determined on the untreated cloth.

The treated cloth is washed in accordance with AATCC Standard Test Method 14-1953 with the following exceptions: (1) the process is run continuously for 120 minutes instead of 60, with a 100 minute wash cycle, (2) sufficient sodium carbonate is added to obtain a pH of 10, (3) steam is injected continuously through the wash cycle to maintain the temperature at 212° F., and (4) the temperature of the first rinse is 160° F. After having been washed according to this procedure and dried, the treated fabric has a wrinkle recovery of 241° (warp plus filling). There is no further loss in wrinkle recovery of the treated fabric after four subsequent washings according to the same procedure. The treated fabric shows less shrinkage after washing than the untreated fabric.

2

The treated fabric is subjected to AATCC Tentative Test Method 69-1958. The test shows essentially no damage to the fabric by retained chlorine.

### Example II

5 An aqueous solution of 6% by weight of bis(beta-methoxyethyl)sulfone and 3% by weight of sodium carbonate (both percentages based on the total weight of the solution) is padded on a cotton print cloth having a count of 80 x 80 to deposit in the cloth 5% by weight of the sulfone, based on the weight of the untreated cloth. The cloth is then dried at 200° F. for 3 minutes and cured at 320° F. for 3 minutes.

The treated fabric is washed for 10 minutes at 100° F. with an aqueous solution of 0.01% by weight of an alkyl aryl sulfonate detergent and 0.01% by weight of tetrasodium pyrophosphate (both percentages based on the total weight of the solution), rinsed at 100° F. for 10 minutes, and then rinsed again at 100° F. for 10 minutes.

10 The treated fabric shows less shrinkage after washing than the untreated fabric and has a wrinkle recovery of 184° (warp plus filling), as determined by ASTM test method D1295-53T, compared to a wrinkle recovery of 100° (warp plus filling) determined on the untreated cloth.

15 The treated fabric is subjected to AATCC Tentative Test Method 69-1958. The test shows essentially no damage to the fabric by retained chlorine.

### Example III

20 An aqueous solution of 8% by weight of bis(beta-methoxyethyl)sulfone and 1% by weight of sodium hydroxide (both percentages based on the total weight of the solution) is padded on a cotton print cloth having a count of 80 x 80 to deposit in the cloth about 7% by weight of the sulfone, based on the weight of the untreated cloth. The cloth is then dried at 200° F. for 3 minutes and cured at 320° F. for 3 minutes.

25 The treated cloth is washed for 10 minutes at 100° F. with an aqueous solution of 0.01% by weight of an alkyl aryl sulfonate detergent and 0.01% by weight of tetrasodium pyrophosphate (both percentages based on the total weight of the solution), rinsed at 100° F. for 10 minutes, and then rinsed again at 100° F. for 10 minutes.

30 The treated fabric shows less shrinkage after washing than the untreated fabric and has a wrinkle recovery of 200° (warp plus filling), as determined by ASTM test method D1295-53T, compared to a wrinkle recovery of 100° (warp plus filling) determined on the untreated cloth.

35 The treated fabric is subjected to AATCC Tentative Test Method 69-1958. The test shows essentially no damage to the fabric by retained chlorine.

35 The textile materials which are treated by the process of this invention are materials containing cellulosic hydroxyl groups, e.g., cotton, rayon, and linen. They may be treated as fabrics or as yarns from which the fabrics are woven.

40 The water-soluble compounds with which the cellulosic textile materials are treated to improve their properties of dimensional stability and wrinkle recovery are compounds corresponding to the general formula:



45 wherein  $\text{R}_1$ ,  $\text{R}_2$ ,  $\text{R}_3$ , and  $\text{R}_4$  are independently selected from the group consisting of  $-\text{H}$ ,  $-\text{CH}_3$ , and  $-\text{C}_2\text{H}_5$ , with the proviso that both radicals of a given "R" designation are the same. Suitable compounds include bis(beta-hydroxyethyl)sulfone, bis(beta-methoxyethyl)sulfone, bis(beta-ethoxyethyl)sulfone, bis(alpha-methyl, beta-hy-

droxyethyl)sulfone, bis(alpha,beta,beta-trimethyl, beta-hydroxyethyl)sulfone, bis(beta-ethyl, beta-hydroxyethyl)sulfone, etc. The amount of water-soluble sulfone treating agent incorporated into the textile material may vary from about 1-20% by weight, based on the weight of the untreated textile material. The amount of water in the treating bath may be varied for ease of operation in incorporating this amount of the treating agent into the textile material.

Treatment of the cellulosic textile materials with the water-soluble sulfone treating agents is accomplished in the presence of an alkaline catalyst. Suitable catalysts are the strongly basic catalysts such as the hydroxides, carbonates, and phosphates of alkali metals, i.e., Li, Na, K, Rb, and Cs; especially preferable are sodium or potassium carbonate and sodium or potassium hydroxide. The aqueous treating bath should contain about 0.5-5% preferably 1-3%, by weight of alkaline catalyst, based on the total weight of the bath.

The process of the invention comprises impregnating a cellulosic textile material with an aqueous solution of the water-soluble sulfone treating agent and an alkaline catalyst, drying the impregnated material, and curing to react the treating agent with the textile material. Impregnation of the textile material with the treating bath can be effected by any of the impregnation techniques commonly used in the textile industry, efficaciously by padding. The impregnated material may be dried at room temperature or at elevated temperatures below curing temperature. Curing is accomplished by heating the dried fabric at temperatures in the range of 250-400° F. for about

0.5-20 minutes, preferably by heating at 300-350° F. for 1-3 minutes, to react the treating agent with the textile material.

The treated textiles obtained by the process of the invention have improved properties of dimensional stability and wrinkle recovery, do not show a tendency toward chlorine retention after bleaching, and do not lose their improved properties when subjected to acid or alkaline hydrolysis.

It is obvious that many variations may be made in the products and processes set forth above without departing from the spirit and scope of this invention.

What is claimed is:

A process which comprises impregnating a cellulosic textile material containing cellulosic hydroxyl groups with an aqueous solution of an alkaline catalyst and bis(beta-methoxyethyl)sulfone.

#### References Cited by the Examiner

##### UNITED STATES PATENTS

|           |         |                |       |         |
|-----------|---------|----------------|-------|---------|
| 2,524,399 | 10/1950 | Schoene et al. | ----- | 8-116   |
| 2,539,704 | 1/1951  | Schoene et al. | ----- | 8-116 X |
| 2,670,265 | 2/1954  | Heyna et al.   | ----- | 8-120 X |
| 2,933,367 | 4/1960  | Reeves et al.  | ----- | 8-120 X |

25

##### FOREIGN PATENTS

779,781 7/1957 Great Britain.

NORMAN G. TORCHIN, Primary Examiner.

30 WILLIAM B. KNIGHT, SAM ROSEN, MORRIS O. WOLK, Examiners.